

## UNITED STATES PATENT OFFICE

2,519,388

## TREATMENT OF FIBROUS CELLULOSIC MATERIALS TO IMPART FLAME RESISTANCE THERETO, COMPOSITIONS THEREFOR, AND PRODUCTS THEREOF

Anne MacMillan Loukomsky, North Plainfield, Roy H. Kienle, Bound Brook, and Theodore F. Cooke, Martinsville, N. J., assignors to American Cyanamid Company, New York, N. Y., a corporation of Maine

No Drawing. Application December 9, 1948,  
Serial No. 64,416

17 Claims. (Cl. 117—137)

**1** This invention relates to a method of imparting flame resistance to a cellulosic material, more particularly a cellulosic material of the class consisting of natural and regenerated celluloses and mixtures thereof, and specifically to a textile comprising fibers of such cellulosic materials, as well as compositions used in such treatments and to the flame-resistant cellulosic products thereof.

Various compounds and compositions have been used or suggested for use as agents for treating fibrous cellulosic and other normally flammable organic materials in order to render them resistant to flame. For a description of such compounds and compositions see the book entitled "Flameproofing Textile Fabrics," edited by Robert W. Little and published in 1947 by Reinhold Publishing Corporation, New York, N. Y., and the references cited therein. Reference also is made to the copending application of one of us (formerly Anne MacMillan, now Anne MacMillan Loukomsky), Serial No. 691,866, filed August 20, 1946, now abandoned, wherein is disclosed and claimed a method of imparting flame resistance to cellulosic textiles which comprises impregnating such textiles with a phosphate of an acyclic amidine, specifically monoguanidine phosphate, and a member of the group consisting of urea, bluret, ammonium cyanate, cyanamide and di-cyandiamide in amounts sufficient to impart flame resistance thereto upon subsequent heating, and then heating the impregnated textiles at a temperature of at least 135° C. to form a washfast, flame-resistant finish therein and thereon.

Agents or treatments for imparting flame resistance to normally flammable organic materials properly may be classified as (1) temporary, (2) semi-durable and (3) permanent or durable, based on their durability in providing continued resistance of the treated textile or other material to flame during use. See page 6 of the aforementioned book by Little for a more complete description of these classes. The present invention is concerned primarily with certain new and useful improvements in the permanent or durable agents or treatments of the kind aforementioned.

The durable treatments heretofore used or suggested have been of three general kinds or types:

1. Urea-phosphate type.
2. Double-bath precipitation type.
3. Metallic oxide-chlorinated body type.

See Little's book, *supra*, pages 179-284, for a complete description and discussion of each of these types. One of the main objections to the urea-

**2** phosphate type of treatment is the tendering effect of the treatment on the cellulosic material whereby its tensile strength is reduced considerably. The double-bath precipitation and the metallic oxide-chlorinated body types of treatments generally yield cellulosic textiles having a harsh or stiff hand, so that the treated textile has a limited field of utility.

The present invention is based on our discovery that fibrous cellulosic materials including those composed solely or comprised mainly (that is, preponderantly by weight) of fibers of natural cellulose (that is, cellulosic materials of natural origin), regenerated cellulose (more particularly viscose rayons) and mixtures thereof can be rendered substantially permanently resistant to flame by suitably treating them with compositions of the kind hereinafter described. Our treated fibrous cellulosic textiles in thread, yarn, fabric or other form are unique in that they are characterized not only by their substantially permanent flame resistance but also by their improved hand or feeling to the touch as compared with the hand of textiles that have been given a double-bath precipitation or a metallic oxide-chlorinated body type of treatment, thereby increasing the field of utility of flame-resistant textiles. Furthermore, these properties are obtained without excessive tendering of the textile, the treated textile in general having a tensile strength (average of the sum of the tensile strength of the warp and filling) of at least 80% of that of the untreated textile when similarly tested for tensile strength, and in many cases a tensile strength which is even higher than that of the untreated textile.

More particularly we have discovered that flame-resistant, fibrous, cellulosic textile materials comprising or composed of fibers of natural cellulose, regenerated cellulose or a mixture thereof and which have a good hand, that is, a hand or feeling to the touch which meets the requirements of the trade, and good tensile strength characteristics are produced by impregnating the normally flammable cellulosic textile with certain materials in particular proportions or ranges of proportions which are critical in carrying the invention into effect. A substantial proportion of the impregnant initially applied is fixedly held by the cellulosic textile after subsequent heat treatment and washing; hence the flame-resistant textiles of our invention properly may be designated as being of the "durable" type or kind.

When the flame-resistant cellulosic textiles of

our invention are tested for flame resistance using a vertical flame test, such as is described herein-after, the "char length" (charred length) ordinarily is not more than about 6 inches, e. g. from 3 to 5½ inches, when the textile material (e. g., cotton cloth or viscose rayon fabric) which has been treated and then subjected to 5 washes in neutral soap solution is one weighing 4 ounces or more per square yard, and not more than about 8 inches, e. g., from 3½ to 7½ inches, when the fabric which has been treated weighs substantially less than 4 ounces, e. g., 2 or 3 ounces per square yard.

In practicing our invention a cellulosic material, more particularly a fibrous cellulose material of the kind defined in the first paragraph of this specification, is impregnated with ingredients comprising (1) a finely divided, oxygen-containing substance of the group consisting of tin, titanium, antimony and bismuth oxides and mixtures thereof and (2) a thermally unstable, halogen-containing thermoplastic substance, more particularly a thermoplastic substance containing at least 20% by weight of combined halogen and capable of rupturing under heat at carbon-halogen bonds, the ingredients of (1) and (2), which together are designated hereinafter as (A), being employed in a weight ratio of 1 part of the former to from 0.6 to 20 parts, more particularly from 0.8 to 4 parts, of the latter. Examples of the thermoplastic substances of (2) that may be employed, alone or in the form of mixtures thereof, are halogen-containing vinyl resins in which not less than 20% by weight of combined halogen is present, for instance, polyvinyl halides (e. g., polyvinyl chloride, polyvinyl bromide, etc.), polyvinylidene halides (e. g., polyvinylidene chloride, polyvinylidene bromide, etc.), copolymers of a vinyl halide and a vinylidene halide (e. g., a copolymer of vinyl chloride and vinylidene chloride), copolymers of a vinyl halide and an acrylic ester (for instance a copolymer of vinyl chloride and an alkyl acrylate (e. g., methyl, ethyl, propyl, butyl, etc., acrylates), halogenated (e. g., chlorinated) paraffins containing not less than 20% by weight of combined halogen, more particularly from about 30 or 40% up to 70 or 75% by weight of combined chloride, bromine, or other halogen, etc. In addition to the ingredients of (1) and (2), other ingredients with which the cellulosic material is impregnated are (3) a water-soluble salt (or mixtures thereof) of an oxygen-containing acid of phosphorus wherein the phosphorus atom has a valence of 5, e. g., a guanidine phosphate, a diguanidine pyrophosphate, diammonium hydrogen phosphate, sodium polyphosphate, ammonium metaphosphate, the mono-, di- and trialkylamine pyrophosphates, etc., and (4) a water-soluble nitrogenous substance of the group consisting of urea, biuret, ammonium cyanate, ammonium dicyanamide and mixtures thereof. The ingredients of (3) and (4), which together are designated hereinafter as (B), are employed in a weight ratio of 1 part of the former calculated as phosphoric acid ( $H_3PO_4$ ) to from 1 to 20 parts, more particularly from 2 to 6 parts of the latter, while the ingredients of (A) and (B) are employed in a weight ratio of 1 part of the former to from 0.2 to 8 parts, more particularly from 1 to 3 parts, of the latter.

The fibrous cellulosic material may be impregnated with the aforementioned ingredients in one or more steps or stages. Thus, it may be impregnated with a dispersion, more particularly

an aqueous dispersion, containing the ingredients mentioned in the preceding paragraph within the ranges of proportions therein specified. The treated cellulosic material is dried at a suitable temperature, e. g., at 40° or 50° to 100° or 105° C., and then heated at a higher temperature within the range of 135° C. (about 135° C.) to 200° C. (about 200° C.). During this latter heat treatment a complex reaction takes place with the result that the finished cellulosic textile in thread, yarn, fabric, felted or other form is rendered substantially permanently resistant to flame, that is to say, the finished textile is resistant to flame even after numerous laundering or dry-cleaning operations. After the heat treatment, the impregnated cellulosic material is washed, e. g., with water, to remove water-soluble substances which are usually present therein.

Alternatively, the fibrous cellulosic material may be impregnated first with an aqueous solution containing a guanidine phosphate or other water-soluble salt of an oxygen-containing acid of phosphorus wherein the phosphorus atom has a valence of 5 (or a mixture of such salts) and one or more of the following: urea, biuret, ammonium cyanate and ammonium dicyanamide. The water-soluble salt of the acid of phosphorus and the urea or other water-soluble nitrogenous substance, which together are designated herein as (B), are employed in ratios by weight within the ranges mentioned hereinbefore. The impregnated fibrous material is dried, heated and washed as described in the preceding paragraph with reference to the one-step process. Thereafter it is treated, as by immersion in a bath containing the same, with a liquid dispersion, more particularly an aqueous liquid dispersion, containing a finely divided metallic oxide or mixture of metallic oxides of the kind aforementioned and, also, a thermally unstable, thermoplastic substance containing at least 20%, preferably at least 40%, of combined chlorine or other halogen and which is capable of rupturing under heat at carbon-halogen bonds, e. g., polymers and copolymers of vinyl chloride. It is important that the metallic oxide or oxides and the halogen-containing thermoplastic substance or substances, which together are designated herein as (A), also be employed in weight ratios within the ranges hereinbefore mentioned. After this second treatment the treated cellulosic material is dried, e. g., by allowing it to stand at room temperature or by heating it at an elevated temperature such, for instance, as at a temperature within the range of 40° or 50° C. up to 100° or 105° C.

From the foregoing description it will be noted that the ingredients of (A) and (B) may be applied to the cellulosic material in one stage (i. e., a one-bath system) or in two stages (i. e., a two-bath system); or, in other words, in the form of at least one and not more than two aqueous liquid compositions containing the same. It is important that the aqueous composition containing the ingredients of (B) have a pH of from about 3 to about 10, more particularly a pH within the range of about 3½ or 4 to about 7 or 8, since at the lower pH values (below about 3) the tensile strength losses in the treated goods are excessive while at the higher pH values (above about 10) the treated textiles have much poorer fire resistance.

Regardless of the method of impregnation of the fibrous cellulosic material with the aforementioned ingredients, it is important that the

ingredients of (A) and (B) be employed in a weight ratio of 1 part of the former to from 0.2 to 8 parts, e. g., from 0.5 to 6 parts, of the latter. In all cases the total amount of the ingredients of (A) and (B) with which the cellulosic material, e. g., a cotton or viscose rayon textile material, initially is impregnated is sufficient to impart flame resistance thereto upon heating within the range of 135° C. to 200° C. and thereafter washing to remove any residual water-soluble substances. Thus, the total amount of the ingredients of (A) and (B) with which the cellulosic material is impregnated advantageously is such that the finished flame-resistant textile contains from about 10% to about 50% by weight (which in some cases may be as high as about 75% by weight when the matter of the hand of the treated material is relatively unimportant), based on the dry weight of the untreated textile, of washfast impregnant.

A preferred method of applying to fibrous cellulosic materials the ingredients used in practicing our invention is in the form of an aqueous dispersion containing the same. The amount of solids in such a dispersion may be varied as desired or as conditions may require, but usually the solids constitute from about 40% to about 70% by weight of the dispersion. A dispersion having excellent storage stability and which is dilutable with water to any desired extent, e. g., to about 50 or 55% by weight of solids, may be prepared, for example, as disclosed and claimed in the copending application of Maurice R. Burnell and William J. Van Loo, Jr., Serial No. 64,418, filed concurrently herewith.

When a two-bath system of applying the ingredients is employed, the first bath is prepared by dissolving in water the proper proportions of (1) guanidine phosphate or other water-soluble salt of an oxygen-containing acid of phosphorus in which the phosphorus atom has a valence of 5 and (2) urea or other water-soluble nitrogenous substance of the group previously described. This bath should be within a pH range of from about 3 to about 10. The bath also may contain a small amount, advantageously not over 7% by weight of the ingredients of (1) and (2), of a polyalkylene polyamine, preferably such a polyamine which is normally a solid or which has a boiling point substantially above 200° C., e. g., triethylene tetramine, tetraethylene pentamine, hexamethylene tetramine, etc. The ingredients are dissolved in water merely by stirring and heating at a suitable temperature, e. g., at 40° C. to 70° C. or higher. The concentration of ingredients in the aqueous bath may be varied as desired or as conditions may require, but usually they constitute from about 30% to about 50% by weight of the aqueous solution. The composition of a typical bath is as follows:

|                         | Approximate per<br>cent by weight |
|-------------------------|-----------------------------------|
| Monoguanidine phosphate | 15.0                              |
| Urea                    | 28.2                              |
| Hexamethylene tetramine | 2.0                               |
| Water                   | 54.8                              |

In preparing the second bath, a dispersion of the finely divided metallic oxide in water is first made with the aid of a suitable dispersing agent, e. g., a sodium, potassium or other alkali-metal salt of a condensation product of an aldehyde, specifically formaldehyde, and a naphthalene sulfonic acid. This dispersion is passed through a colloid mill in order to reduce the average

particle size to one micron or less. To the resulting dispersion is then added a dispersion of a polyvinyl halide polymerization product, more particularly a polyvinyl chloride polymerization product, e. g., polyvinyl chloride itself or a vinyl chloride copolymer comprising mainly vinyl chloride, for instance a copolymer of, by weight, 80 to 99% of vinyl chloride (in the copolymer molecule) and 20 to 1% of vinylidene chloride, a lower alkyl acrylate (e. g., methyl, ethyl, etc., acrylates), or a vinyl ester of an aliphatic monocarboxylic acid (e. g., vinyl acetate, vinyl propionate, etc.) or other thermoplastic substance containing at least 20% by weight of combined halogen and capable of rupturing under heat at carbon-halogen bonds. The mixture is thoroughly agitated until a homogeneous liquid composition or dispersion is obtained. The concentration of solids in this dispersion may be varied as desired or as conditions may require, but usually they constitute from about 10% to about 30% by weight thereof.

Any suitable apparatus may be employed in applying the treating composition (used in a one-bath process) or compositions (used in a two-bath process) to the cellulosic material. For example, the dry or substantially dry cellulosic textile to be treated may be immersed in the aqueous composition or compositions and then passed through pressure rolls, mangles or centrifugal extractors to secure uniform impregnation and a controlled removal of the excess material. The cellulosic textile in fabric or other form also may be impregnated by other methods, e. g., by spraying. The wet pick-up of the composition (one-bath process) or compositions (two-bath process) by the textile may range, for example, between about 50% and about 150% by weight of the textile undergoing treatment.

The pick-up of the treating agent by the cellulosic textile material, regardless of whether the said agent is applied in one or two distinct steps or stages, is adjusted so that the finished textile contains from about 10 to about 75%, usually from 10 to 50% by weight, based on the dry weight of the untreated textile, of washfast impregnant. As has been indicated hereinbefore, when the matter of hand of the finished textile is important, it generally contains not more than about 50%, e. g., from 10 or 15% to 30 or 40%, based on the dry weight of the untreated textile, of washfast impregnant.

After impregnating the cellulosic textile with an aqueous dispersion containing the ingredients of both (A) and (B) or with a solution containing the ingredients of (B) only, the treated material is dried to remove most or substantially all of the liquid present therein, after which it is heated at a higher temperature of the order of about 135° C. to about 200° C. During this latter heat treatment a substantial loss of solids takes place, which may be as much as one-half to two-thirds of the total weight of the ingredients of (B) with which the cellulosic material initially was impregnated. Hence, in order to obtain a finished textile containing from 10 to 50% or, in those cases where desired up to 65 or 75% by weight, based on the dry weight of the untreated textile, of washfast impregnant, the amount of solids in the textile as initially impregnated should be sufficiently high to allow for this weight loss of solids during the heat-treating and washing steps.

In order that those skilled in the art better may understand how the present invention may

be carried into effect, the following examples are given by way of illustration and not by way of limitation. All parts and percentages are by weight.

#### EXAMPLE 1

This example illustrates the preparation and use of a single-bath or "pad liquor" in carrying the present invention into effect.

#### Preparation of a dispersion of antimony trioxide

A small amount of dispersing agent, more particularly 13 parts of the sodium salt of a condensation product of formaldehyde and a naphthalene sulfonic acid (Tanol P) is dissolved in 577 parts of water. Under rapid stirring with a homogenizing type of mixer, 410 parts of finely divided antimony trioxide is added to the solution. The resulting dispersion is then passed through a colloid mill to reduce the particle size to 1 micron or less.

#### Preparation of pad liquor

A typical formula for the preparation of the pad liquor is as follows:

|                                                                                                                                                                        | Parts |
|------------------------------------------------------------------------------------------------------------------------------------------------------------------------|-------|
| Monoguanidine phosphate                                                                                                                                                | 151   |
| Urea                                                                                                                                                                   | 282   |
| Hexamethylene tetramine                                                                                                                                                | 20    |
| Water                                                                                                                                                                  | 320   |
| Antimony trioxide dispersion (prepared as described above)                                                                                                             | 136   |
| Aqueous dispersion containing 55-56% by weight of an unplasticized vinyl chloride copolymer containing between 80 and 95% by weight of vinyl chloride in the copolymer | 91    |

The monoguanidine phosphate, urea and hexamethylene tetramine are added to the water and dissolved therein by heating at 40°-50° C. The aqueous dispersion of the antimony trioxide is added to the aqueous dispersion of the vinyl chloride copolymer, and are thoroughly mixed together. (The aqueous dispersion of the vinyl chloride copolymer may be, and preferably is, the product which is available from the B. F. Goodrich Chemical Company, Akron, Ohio, under the trade name of "Geon Latex X-15.") The resulting dispersion is added to the solution of the other ingredients, and the mass is well mixed to form a substantially homogeneous liquid composition which constitutes the pad liquor.

The vinyl chloride copolymer used in the above aqueous dispersion and in dispersions referred to in other examples which follow, may be, for example, a copolymer of, by weight, about 80% to about 95%, e. g., about 85 to 90% of vinyl chloride and about 20% to about 5%, e. g., about 15% to 10%, of an alkyl acrylate, more particularly a lower alkyl acrylate such, for instance, as methyl, ethyl, propyl or butyl acrylate.

#### Treatment of fabrics

A cellulosic fabric such, for example as cotton cloth or a viscose rayon fabric is immersed in the pad liquor and immediately passed through two rubber squeeze rolls, the pressure being adjusted so that the so-called "wet pick-up" of pad liquor by the fabric is approximately 120% by weight of the dry, untreated fabric. After drying the untreated fabric, e. g., by heating at 60°-70° C., the dried fabric is heated at 160° C. for from 10 to 15 minutes. Thereafter the fabric is rinsed well in water to remove residual water-

soluble substances therefrom, and again is dried (for instance at about 60°-70° C.).

#### EXAMPLE 2

This example illustrates the preparation and use of two baths in carrying our invention into effect.

#### Bath 1

|                         | Parts |
|-------------------------|-------|
| Monoguanidine phosphate | 150   |
| Urea                    | 282   |
| Hexamethylene tetramine | 20    |
| Water                   | 548   |

The above-named solid ingredients are dissolved in the water by stirring and heating at 40°-50° C.

#### Bath 2

|                                                                                                                                         | Parts |
|-----------------------------------------------------------------------------------------------------------------------------------------|-------|
| Aqueous dispersion containing 55-56% by weight of a vinyl chloride copolymer such as described under Example 1                          | 199   |
| Finely divided antimony trioxide                                                                                                        | 58    |
| Dispersing agent, more particularly the sodium salt of a condensation product of formaldehyde and a naphthalene sulfonic acid (Tanol P) | 2     |
| Water                                                                                                                                   | 741   |

The dispersing agent is dissolved in one-half of the water and the finely divided antimony trioxide is added thereto under rapid stirring with a turbo-type mixer. The resulting dispersion is passed through a colloid mill in order to reduce the particle size to 1 micron or less. The aqueous dispersion of the vinyl chloride copolymer is diluted with the remainder of the water, the antimony trioxide dispersion added thereto, and the mass is well mixed to form a substantially homogeneous liquid composition.

#### Treatment of fabrics

The same procedure is followed in treating a cellulosic fabric with the ingredients of Bath 1 as is described under Example 1. The treated, rinsed and dried fabric is then immersed in Bath 2 and immediately passed through rubber squeeze rolls, the pressure of which is adjusted so that the wet pick-up of the dispersion by the fabric is approximately 100% by weight of the dry fabric resulting from the initial treatment. The wet fabric is dried at a suitable temperature, e. g., by heating at 60°-70° C. The flame resistance of the treated fabric is of the same general order as that of fabrics which have been treated by the one-bath process described under Example 1.

Examples 3 to 16, inclusive, which follow, are illustrative of further variations in the ingredients and proportions thereof that may be used in the preparation of the treating compositions of our invention and of their use in imparting flame-resisting characteristics to cotton fabrics and rayon fabrics (other than cellulose ester rayon fabrics), using both one-bath and two-bath processes. The procedure, in general, was as follows in the case of Examples 3 to 11, inclusive, 15 and 16, wherein the cellulosic material treated was 80 x 80 cotton cloth.

#### Preparation of pad liquor

##### A. FOR ONE-BATH PROCESS

75 A dispersion of the finely divided metallic

oxide was prepared as follows unless otherwise specified:

|                                                    | Parts |
|----------------------------------------------------|-------|
| Finely divided metallic oxide                      | 41.0  |
| Dispersing agent such as described under Example 2 | 1.3   |
| Water                                              | 57.7  |

The dispersing agent was dissolved in the water, and the finely divided metallic oxide was incorporated slowly therein under high-speed stirring. After all the metallic oxide had been dispersed, the dispersion was passed through a colloid mill (clearance: 0.002 inch). The particle size of the dispersed solid was, for the most part, one micron or less. Aggregates having a particle size up to 3 microns may be present in the dispersion.

The water-soluble salt of the oxygen-containing acid of phosphorus and the water-soluble nitrogenous substance, which ingredients are more specifically identified in the various tables which follow, were dissolved in water, using heat if necessary to effect solution. The above dispersion of the finely divided metallic oxide and the dispersion of a thermally unstable, thermoplastic substance containing at least 20% of combined halogen and capable of rupturing under heat at carbon-halogen bonds, e. g., a vinyl chloride polymerization product, more particularly a vinyl chloride copolymer of the kind described under Example 1, were then added to the solution of the other two ingredients, and the resulting mixture was thoroughly agitated to obtain a substantially homogeneous aqueous dispersion.

#### B. FOR TWO-BATH PROCESS

The first bath comprises an aqueous solution of the water-soluble nitrogenous substance and the water-soluble salt of the oxygen-containing acid of phosphorus. The second bath contains the dispersion of finely divided metallic oxide and of the halogen-containing thermoplastic substance.

##### *Application to fabrics*

###### A. USING ONE-BATH PROCESS

Weighed strips of the cotton fabric were impregnated with the pad liquor and passed between rubber squeeze rolls. The pressure on the rolls was adjusted so that a wet pick-up of not less than 110%, unless otherwise stated, was obtained; that is, the weight of the aqueous dispersion picked up, expressed as a percentage of the weight of the dry fabric, was not less than 110%. The treated fabrics were dried at 60°-80° C. and then heated at a higher temperature in a forced-draft oven. The heated fabrics were thoroughly rinsed for 10 minutes in a container into which water was running. The fabric was dried at 60°-80° C. and again weighed after allowing it to stand for at least one hour in free contact with the atmosphere. The per cent "add-on" was determined by subtracting the initial dry weight from the final dry weight after rinsing, and dividing the difference by the initial dry weight and multiplying the quotient by 100.

###### B. USING TWO-BATH PROCESS

The pad liquor of the first bath was applied to the fabric in exactly the same manner as in the one-bath process. The add-on, in general, was at least 15% by weight of the dry fabric (80 x 80 cotton) unless otherwise specified. If

less than 15% add-on was obtained, the entire application procedure was repeated on the fabric, using the same bath, until the add-on was 15% or more, based on the dry weight of the fabric.

The pad liquor of the second bath was applied to the fabric (pretreated as described above), using a wet pick-up of 100-125% unless otherwise specified and drying at 60°-80° C.

##### *Washing procedure*

A small oscillating washing machine was used to wash the flame-resistant fabrics unless otherwise specified. A one-pound load was used for each wash and the fabrics were washed for 15-minute intervals using 12 liters of 0.5% neutral soap solution at 65°-75° C. They were spun and rinsed for from 3 to 5 minutes in lukewarm water, spun and then rinsed further by hand. Flame tests were made after washing once and five times unless otherwise indicated.

##### *Flame tests*

Flame tests were made using a specially constructed apparatus and a procedure which followed in general that given in ASTM Tentative Specifications Designation: D626-41T, issued 1941. Samples 2½ inches by 10 inches were cut with the long dimension parallel to the warp and others parallel to the fill. The apparatus consisted of a hood, a shield around the test piece, a Bunsen burner and a holder for the sample. The fabric to be tested was suspended vertically in the shield, which was placed in a hood with the fan off, the fabric being suspended in the shield by means of a clamp at the top and bottom. The door of the hood was then closed. The burner had previously been regulated to a luminous flame 1½ inches high, and was placed under the suspended sample so that the end of the sample extended ¾ inch into the flame. The flame was held under the sample for 12 seconds and then extinguished. The duration of after-flaming of the sample was measured by means of a stop watch. Any tendency of the sample to after-glow or smoke was noted and timed if possible. The total length of char in inches was measured by the tear length produced with a tearing weight equal to approximately 10% of the tearing strength of the unburned fabric.

The pH of the bath of pad liquor (pH of Bath 1 in the case of a two-bath process) as well as the pH of rinsings from the treated fabric after having been heated at between 135° C. and 200° C. (that is, the so-called "cured" fabric) were determined electrometrically with glass and calomel electrodes. The rinsings were prepared by soaking the cured fabric in a small volume of distilled water and squeezing out the excess liquid. This liquid was used in testing for pH. The fabric was then rinsed again in a large volume of running water.

In some cases the tensile strength of the treated fabrics was measured with a pendulum tester, following the strip methods of Federal Specification CCC-T-191a. Ravelled strips (one-inch wide) as well as one-inch treated cotton tape were tested.

##### EXAMPLE 3

In this example various water-soluble salts of an oxygen-containing acid of phosphorus, wherein the phosphorus atom has a valence of 5, were employed. The water-soluble nitrogenous substance was urea, the metallic oxide was antimony

## 11

trioxide, and the halogen-containing thermoplastic substance was a vinyl chloride copolymer such as that described under Example 1, more particularly an unplasticized copolymer of, by weight, about 85% of vinyl chloride and about 15% of an alkyl acrylate. The ingredients, which were applied by both a one-bath and a two-bath proc-

## 12

soluble salt in the case of the two-bath process were dried at 60°-80° C. and then cured by heating for 15 minutes at 160° C. In the tables which follow, "0" under the heading "Bath 2" indicates that the treatment was by a one-bath process.

Further information on the treatment and on the results obtained are given in Table I.

Table I

|                                    | Weight Ratio of Urea to— |                   | Percent Total Dry Add-On |        | pH Bath | pH Rinsings | Avg. Percent Tensile Strength Loss or Gain | Flame Test |          |        |          |
|------------------------------------|--------------------------|-------------------|--------------------------|--------|---------|-------------|--------------------------------------------|------------|----------|--------|----------|
|                                    |                          |                   | Bath 1                   | Bath 2 |         |             |                                            | 1 Wash     | 5 Washes | 1 Wash | 5 Washes |
|                                    | Salt as Such             | Salt as $H_3PO_4$ |                          |        |         |             |                                            |            |          |        |          |
| Monoguanidine phosphate.           | 1:1                      | 1:0.6             | 29                       | 0      | 4.2     |             | -6                                         | 4%         | 4%       |        |          |
| Do.                                | 1:1.5                    | 1:0.95            | 34                       | 0      | 4.2     |             | -7                                         | 2%         | 4%       |        |          |
| Do.                                | 1:1.8                    | 1:1.1             | 21                       | 18     | 4.2     |             |                                            | 5          | 5%       | 3      | 11       |
| Do.                                | 5:1                      | 8:1               | 27                       | 0      | 4.6     |             | -2                                         | 4%         | 4%       | 4      | 12       |
| Do.                                | 9:1                      | 14:1              | 30                       | 0      | 4.8     |             | +4                                         | 4%         | 4%       | 6      | 22       |
| Do.                                | 12:1                     | 19:1              | 23                       | 0      | 4.8     |             |                                            | 3%         | 3%       | 5      | 16       |
| Diguanidine phosphate.             | 2:1                      | 4:4:1             | 15.5                     | 19     | 8.8     | 8.4         |                                            | 3%         | 3%       | 3      | 18       |
| Do.                                | 1:2:2                    | 1:1               | 16                       | 19     | 8.5     | 8.4         |                                            | 3%         | 3%       | 3      | 11       |
| Do.                                | 8:7:1                    | 19:1              | 19                       | 19     | 8.3     | 6.6         |                                            | 4          | 3%       | 3      |          |
| Diguanidine pyrophosphate.         | 1:2                      | 1:1.3             | 20                       | 17     |         |             | -4                                         | 4%         | 5%       |        | 10       |
| Do.                                | 2:1                      | 3:1               | 30                       | 0      |         |             | -7                                         | 4%         | 4%       | 4      |          |
| Do.                                | 5:1                      | 7.5:1             | 24                       | 0      |         |             | -4                                         | 4%         | 5        |        |          |
| Do.                                | 8:1                      | 12:1              | 21.5                     | 0      |         |             | -2                                         | 4          | 3%       |        |          |
| Do.                                | 9:1                      | 13.5:1            | 20                       | 0      |         |             | -7                                         | 4%         | 4%       | 5      |          |
| Do.                                | 1:2                      | 1:1.3             | 23                       | 15     |         |             | -15                                        | 4%         | 4%       | 4      |          |
| Do.                                | 2:1                      | 3:1               | 32                       | 0      |         |             |                                            | 4%         | 4%       |        |          |
| Do.                                | 6:1                      | 7.5:1             | 24.5                     | 0      |         |             | -2                                         | 3%         | 4%       |        |          |
| Do.                                | 8:1                      | 12:1              | 22                       | 0      |         |             |                                            | 3%         | 4%       | 7      | 57       |
| Do.                                | 12:1                     | 18:1              | 21                       | 0      | 3.5     |             |                                            | 5%         | 4%       | 4      |          |
| Do.                                | 9:1                      | 13.5:1            | 21                       | 0      |         |             | +8                                         | 4%         | 4%       |        |          |
| Guanylurea phosphate.              | 1:2                      | 1:1               | 20                       | 16     |         |             | -3                                         | 4%         | 4%       |        | 13       |
| Do.                                | 2:1                      | 4:1               | 27                       | 0      |         |             | -15                                        | 4          | 4%       |        |          |
| Do.                                | 5:1                      | 10:1              | 21                       | 0      |         |             | -14                                        | 4%         | 4%       |        |          |
| Do.                                | 8:1                      | 16:1              | 14.5                     | 0      |         |             | +1                                         | 3%         | 4%       |        |          |
| Do.                                | 9:1                      | 18:1              | 29                       | 0      |         |             | +6                                         | 4          | 4%       | 4      | 11       |
| Biguanide phosphate.               | 1:1.6                    | 1:8               | 24                       | 17     | 7.2     | 7.1         |                                            | 3%         | 4%       | 2      | 23       |
| Do.                                | 2:1                      | 4:1               | 36                       | 0      | 7.6     |             | -13                                        | 4%         | 4%       |        |          |
| Do.                                | 8:1                      | 16:1              | 25                       | 0      | 7.6     |             | -5                                         | 3%         | 4%       |        | 17       |
| Do.                                | 9:1                      | 18:1              | 32                       | 0      | 7.6     |             | -8                                         | 4%         | 4%       |        |          |
| $Na_2HPO_4$ .                      | 1:1.2                    | 1:1               | 15                       | 20     | 4.2     | 6.3         |                                            | 3          | 4%       | 3      | 26       |
| $Na_2HPO_4$ .                      | 5:1                      | 6:1               | 32                       | 0      | 4.4     |             |                                            | 3%         | 4%       | 7      | 25       |
| $Na_2HPO_4$ .                      | 9:1                      | 11:1              | 30                       | 0      | 4.6     |             | -15                                        | 4%         | 5%       | 7      | 22       |
| $Na_2HPO_4$ .                      | 16:3:1                   | 20:1              | 17                       | 20     | 5.3     | 6.1         |                                            | 3          | 4%       | 3      | 10       |
| $Na_2HPO_4 \cdot 12H_2O$ .         | 2:1                      | 7.3:1             | 21                       | 0      | 9.3     |             | -3                                         | 3%         | 4%       |        | 50       |
| $Na_2HPO_4 \cdot 12H_2O$ .         | 3:7:1                    | 13.5:1            | 19                       | 0      | 9.3     |             | +24                                        | 5%         | 5%       |        | 12       |
| $Na_2HPO_4 \cdot 12H_2O$ .         | 4:8:1                    | 17.6:1            | 23                       | 0      | 9.3     |             | +12                                        | 3%         | 3%       |        | 75       |
| $Na_2HPO_4 \cdot 12H_2O$ .         | 9:1                      | 33:1              | 23                       | 0      | 9.3     |             | +7                                         | 4%         | 4%       |        |          |
| $K_2HPO_4$ .                       | 11:2:1                   | 20:1              | 19                       | 20     | 6.9     | 6.6         |                                            | 4%         | 4%       | 1      | 7        |
| $K_2HPO_4$ .                       | 1:1.78                   | 1:1               | 21                       | 20     | 7.7     | 8.2         |                                            | 4          | 3%       | 2      | 6        |
| $(NH_4)_2HPO_4$ .                  | 1:1.35                   | 1:1               | 18                       | 18     | 8.1     | 3.8         |                                            | 3%         | 3%       | 5      | 14       |
| $(NH_4)_2HPO_4$ .                  | 4:7:1                    | 6:1               | 17                       | 21     |         |             |                                            | 5%         | 5%       | 26     | 11       |
| $(NH_4)_2HPO_4$ .                  | 14:8:1                   | 19.4:1            | 16                       | 22     | 7.7     | 5.8         |                                            | 4%         | 4%       | 6      | 10       |
| $Na_2HPO_4 \cdot 2H_2O$ .          | 18:5:1                   | 20:1              | 29.3                     | 0      | 6.5     | 5.9         |                                            | 4          | 4%       | 5      | 10       |
| $Na_2PO_4$ .                       | 5:1                      | 5.2:1             | 11                       | 19     |         |             | -14                                        | 4%         | 5        |        |          |
| $Na_2PO_4$ .                       | 8:1                      | 8.3:1             | 17                       | 0      |         |             | -3                                         | 4%         | 6        |        |          |
| Sodium polyphosphate.              | 5:1:1                    | 5.8:1             | 50                       | 0      | 3.2     |             | -7                                         | 5%         | 5%       | 2      | 35       |
| Ammonium polyphosphate.            | 2:8:1                    | 3:1               | 38                       | 0      | 2.4     | 4.1         |                                            | 5%         | 5%       | 0      | 5        |
| $(CN_3NH_2)_2 \cdot 2H_2PO_4$ .    | 2:1                      | 2.6:1             | 14                       | 19     |         |             |                                            | 3%         | 3%       | 2      | 23       |
| $(CH_3NH_2)_2 \cdot 2H_2PO_4$ .    | 18:1                     | 23.5:1            | 15                       | 20     | 6.0     | 5.7         |                                            | 3%         | 4        |        | 14       |
| $(CH_3NH_2)_2 \cdot 2H_2PO_4$ .    | 0.9:1                    | 1.2:1             | 16                       | 19     | 5.1     | 3.6         |                                            | 3%         | 3%       | 4      | 8        |
| Ethylenediamine polyphosphate.     | 0.83:1                   | 1:1               | 19                       | 18     | 3.4     | 3.5         |                                            | 4%         | 4%       | 0      | 8        |
| Do.                                | 16.5:1                   | 20:1              | 16                       | 20     | 8.2     | 5.5         |                                            | 3          | 3%       | 4      | 12       |
| Primary cyclohexylamine phosphate. | 2:1                      | 4:1               | 15                       | 18     |         |             |                                            | 4          | 4%       | 3      | 22       |
| Primary morpholine phosphate.      | 2:1                      | 3.8:1             | 13                       | 19     |         |             |                                            | 4%         | 5        | 2      | 26       |
| Secondary pyridine phosphate.      | 2:1                      | 5.2:1             | 11                       | 19     |         | 5.7         |                                            | 4%         | 4%       | 5      | 47       |

NOTE.—The polyphosphoric acid, from which the polyphosphates employed in this and other examples were made, comprised, by weight, about 3-8% orthophosphoric acid, about 32-50% metaphosphoric acid and about 47-60% pyrophosphoric acid. It assayed 82-84%  $P_2O_5$ .

ess as hereinbefore described, were used in the following weight percentages:

## Per cent

|                             |      |
|-----------------------------|------|
| Urea plus salt <sup>1</sup> | 43.3 |
| Antimony trioxide           | 5.8  |
| Vinyl chloride copolymer    | 11.0 |
| Water                       | 39.9 |

70

<sup>1</sup> The weight ratio of urea to salt as salt and, also, to the latter calculated as  $H_3PO_4$  as shown in Table I.

The treated textiles after immersion in the treating composition of the one-bath process or after immersion in the first bath containing the water-

EXAMPLE 4

65 In this example the water-soluble salt of an oxygen-containing acid of phosphorus was monoguanidine phosphate. The other ingredients were the same as in Example 3. The antimony trioxide and the vinyl chloride copolymer were used in varying amounts and, also, in varying weight ratios of the one to the other. A small amount of a buffering agent, more particularly a polyalkylene polyamine and specifically hexamethylene tetramine, also was employed. Both one-bath and two-bath application methods were used. Fur-

ther details on weight percentages of ingredients are shown below:

|                          | Per cent     |  |
|--------------------------|--------------|--|
| Urea                     | 28.2         |  |
| Monoguanidine phosphate  | 15.0         |  |
| Hexamethylene tetramine  | 2.0          |  |
| Antimony trioxide        | See Table II |  |
| Vinyl chloride copolymer | See Table II |  |
| Water                    | Remainder    |  |

Further information on the treatment and on the results obtained are given in Table II.

#### EXAMPLE 6

In this example varying amounts of ammonium dicyanamide, ammonium cyanate and bluret were used either wholly in place of urea or in combination with urea in the case of bluret, the other ingredients being monoguanidine phosphate, antimony trioxide and a vinyl chloride copolymer such as was employed in the prior examples. Table IV shows the ratios of ammonium dicyanamide, ammonium cyanate and of bluret plus urea to monoguanidine phosphate as such and

Table II

| Weight Ratio<br>$Sb_2O_3$ to<br>Copolymer | Per Cent<br>$Sb_2O_3$<br>in Bath | Per Cent<br>Vinyl<br>Chloride<br>Copolymer<br>in Bath | Per Cent Total Dry<br>Add-On |        | pH<br>Bath | pH<br>Rinsings | Avg. Per<br>Cent<br>Tensile<br>Strength<br>Loss | Flame Test Vertical<br>Charred Length,<br>Inches |          | Time After Glow,<br>Sec. |          |
|-------------------------------------------|----------------------------------|-------------------------------------------------------|------------------------------|--------|------------|----------------|-------------------------------------------------|--------------------------------------------------|----------|--------------------------|----------|
|                                           |                                  |                                                       | Bath 1                       | Bath 2 |            |                |                                                 | 1 Wash                                           | 5 Washes | 1 Wash                   | 5 Washes |
|                                           |                                  |                                                       | 1.75:1                       | 10.6   | 6.1        | 18             | 17                                              | 3½                                               | 4½       |                          |          |
| 1.5:1                                     | 8.4                              | 5.55                                                  | 18                           | 14     |            |                | —7                                              | 3                                                | 3½       |                          |          |
| 1:5                                       | 1.75                             | 8.9                                                   | 33                           | —      |            |                | 5                                               | 4½                                               | 2        | 5                        |          |
| 1:10                                      | 0.96                             | 9.7                                                   | 32                           | —      |            |                | 5                                               | 4½                                               | 2        | 9                        |          |
| 1:20                                      | 0.48                             | 10.2                                                  | 34                           | —      |            |                | 4½                                              | 4½                                               | 0        | 0                        |          |
| 1:40                                      | 0.23                             | 10.2                                                  | 32                           | —      | 6.9        | 6.0            | 3½                                              | 3½                                               | 0        | 0                        | 3        |

#### EXAMPLE 5

In this example the ingredients employed were the same as in Example 4. The weight ratio of antimony trioxide to vinyl chloride copolymer was 1.1:1, these ingredients together being designated as "A." The weight ratio of urea to monoguanidine phosphate was 2:1, while the weight

calculated as  $H_3PO_4$ . The ingredients were applied by a two-bath process, the second bath being an aqueous dispersion containing, by weight, 5.8% of  $Sb_2O_3$  and 11% of the aforementioned copolymer. Further information on the treatment and on the results obtained also appears in Table IV.

Table IV

| Nitrogenous Substance            | Weight Ratio of<br>Nitrogenous<br>Substance to— |                      | Percent Total<br>Dry Add-On |        | pH<br>Bath | pH<br>Rinsings | Flame Test |          |        |          |  |  |
|----------------------------------|-------------------------------------------------|----------------------|-----------------------------|--------|------------|----------------|------------|----------|--------|----------|--|--|
|                                  | Salt as<br>Such                                 | Salt as<br>$H_3PO_4$ | Bath 1                      | Bath 2 |            |                | 1 Wash     | 5 Washes | 1 Wash | 5 Washes |  |  |
|                                  |                                                 |                      |                             |        |            |                |            |          |        |          |  |  |
| Ammonium dicyanamide...          | 12.5:1                                          | 20:1                 | 19                          | 20     | 4.8        | 5.5            | 3½         | 5        | 4      | 14       |  |  |
| Do...                            | 1:1.6                                           | 1:1                  | 18                          | 19     | 4.2        | 3.3            | 3½         | 3½       | 3      | 3        |  |  |
| Ammonium cyanate...              | 12.5:1                                          | 20:1                 | 16                          | 20     | 9.1        | 7.5            | 3½         | 3½       | 3      | 17       |  |  |
| Do...                            | 1:1.6                                           | 1:1                  | 21                          | 18     | 6.1        | 6.3            | 3½         | 3½       | 9      | 11       |  |  |
| Bluret and urea <sup>1</sup> ... | 1:1.6                                           | 1:1                  | 20                          | 17     | 5.1        | 5.7            | 4½         | 4½       | 0      | 20       |  |  |

<sup>1</sup> Urea was present to such an extent as to make the sum of the urea and bluret equal to about 40% by weight of an aqueous solution thereof, the solution (without the urea) having first been saturated at 90° C. with bluret.

ratio of urea to hexamethylene tetramine was 7.5:1. The urea, monoguanidine phosphate and hexamethylene tetramine together are designated as "B." The weight ratios of A to B were varied as shown in Table III, which also gives further information on the treatment and on the results obtained.

Table III

| Weight<br>Ratio of<br>A:B | Per Cent Dry<br>Total Add-On |        | Avg. Per<br>Cent Tensile<br>Strength<br>Loss<br>or Gain | Flame Test Vertical<br>Charred Length,<br>Inches |          | 1 Wash | 5 Washes |
|---------------------------|------------------------------|--------|---------------------------------------------------------|--------------------------------------------------|----------|--------|----------|
|                           | Bath 1                       | Bath 2 |                                                         | 1 Wash                                           | 5 Washes |        |          |
| 5:1                       | 4                            | 59     | +12                                                     | 4                                                | 4½       |        |          |
| 1:1                       | 20                           | 53     | -14                                                     | 3½                                               | 3½       |        |          |
| 1:5                       | 22                           | —      | -7                                                      | 3                                                | 4½       |        |          |

In this example a different halogen-containing thermoplastic substance, more particularly a chlorinated paraffin containing about 60% by weight of combined chlorine, was used in place of a vinyl chloride copolymer. Further details on weight percentages of ingredients are given below:

|                                                                             | Per cent |
|-----------------------------------------------------------------------------|----------|
| Urea                                                                        | 28.2     |
| Monoguanidine phosphate                                                     | 15.1     |
| Antimony trioxide                                                           | 15.0     |
| Chlorinated paraffin containing about 60%<br>by weight of combined chlorine | 15.0     |
| Water                                                                       | 26.7     |

The ingredients were applied by a two-bath process as hereinbefore described. Further information on the treatment and on the results obtained are given in Table V.

| Weight Ratio of Chlorinated Paraffin to Sb <sub>2</sub> O <sub>3</sub> | Per Cent Dry Total Add-On |        | Flame Test                      |          |        |                       |  |  |
|------------------------------------------------------------------------|---------------------------|--------|---------------------------------|----------|--------|-----------------------|--|--|
|                                                                        |                           |        | Vertical Charred Length, Inches |          |        | Time After Glow, Sec. |  |  |
|                                                                        | Bath 1                    | Bath 2 | 1 Wash                          | 5 Washes | 1 Wash | 5 Washes              |  |  |
| 1:1                                                                    | 26                        | 32     | 4                               | 4½       | 2      | 27                    |  |  |

## EXAMPLE 8

This example illustrates the use of a dispersion containing the essential ingredients, which dispersion was stabilized with ammonium hydroxide as more fully described in the aforementioned copending application of Maurice R. Burnell and William J. Van Loo, Jr., Serial No. 64,418. It

15 latex which was employed in each of the previous examples. The ingredients were applied by a one-bath process. For additional details of the treatment employed and the results obtained, see Table VII. The percentage proportions shown in this table refer to the per cent of each ingredient in the aqueous bath, water constituting the remainder of the bath.

Table VII

| Percent Mono-guanidine Phosphate | Percent Urea | Percent Hexamethylene Tetramine | Sodium Salt of Condensation Product of HCHO and a Naphthalene Sulfonic Acid | Vinyl Chloride Copolymer | Percent Bismuth Trioxide | Percent Stannic Oxide | Percent Dry Add-On | pH Bath | pH Rinsings | Flame Tests                     |                       |        |          |
|----------------------------------|--------------|---------------------------------|-----------------------------------------------------------------------------|--------------------------|--------------------------|-----------------------|--------------------|---------|-------------|---------------------------------|-----------------------|--------|----------|
|                                  |              |                                 |                                                                             |                          |                          |                       |                    |         |             | Vertical Charred Length, Inches | Time After Glow, Sec. | 1 Wash | 5 Washes |
| 15.1                             | 28.2         | 2                               | 0.18                                                                        | 5.1                      | 5.6                      | —                     | 31                 | —       | —           | 4½                              | 4½                    | —      | —        |
| 15.1                             | 28.2         | —                               | 0.18                                                                        | 5.1                      | —                        | 5.6                   | 32                 | 4.7     | 7.2         | —                               | —                     | 0      | 4        |

35 was diluted with one-half its weight of water prior to use in a one-bath process. The vinyl chloride copolymer was used in the form of an aqueous dispersion containing about 55 to 56% by weight of the same, the product employed being, as in the preceding examples, the aforementioned material which is available under the trade name of "Geon Latex X-15" and in which the halogen-containing thermoplastic substance may be described more particularly as an unplasticized copolymer of vinyl chloride and an alkyl acrylate in a ratio, by weight, of from about 80 to about 95 parts of the former to from about 20 to about 5 parts of the latter. Further information on the treatment and on the results obtained are given in Table VI.

## EXAMPLE 10

35 This example illustrates the use of still another metallic oxide, specifically titanium dioxide, in the treating compositions. Both one-bath and two-bath processes were employed in applying the ingredients to 80 x 80 cotton cloth. Further details on weight percentages of ingredients are given below:

40 Per cent  
Urea ----- 28.2  
Monoguanidine phosphate ----- 15.1  
Hexamethylene tetramine ----- 2.0  
45 Titanium dioxide ----- See Table VIII  
Vinyl chloride copolymer such as  
was used in prior examples ... See Table VIII  
Water ----- Remainder

Table VI

| Monoguanidine Phosphate | Composition of Mix in Parts by Weight |                                |                                                                                         |                          |       |                                 | Per Cent Dry Add-On | Ratio Weight of Mix to Water in Pad Liquor | pH Bath | pH Rinsings | Avg. Per Cent Tensile Strength Loss | Flame Test |          |        | Remarks                                                                    |
|-------------------------|---------------------------------------|--------------------------------|-----------------------------------------------------------------------------------------|--------------------------|-------|---------------------------------|---------------------|--------------------------------------------|---------|-------------|-------------------------------------|------------|----------|--------|----------------------------------------------------------------------------|
|                         | Urea                                  | Sb <sub>2</sub> O <sub>3</sub> | Sodium Salt of a Condensation Product of HCHO and a Naphthalene Sulfonic Acid (Tamil P) | Vinyl Chloride Copolymer | Water | Vertical Charred Length, Inches |                     |                                            |         |             |                                     | 1 Wash     | 5 Washes | 1 Wash | 5 Washes                                                                   |
| 40-----                 | 200                                   | 5.0                            | 0.16                                                                                    | 45                       | 43    | 2:1                             | 23                  | 5.1                                        | 6.3     | —14         | 6                                   | 6          | 2        | 35     | Fresh mix-dissolved soluble portion by warming and stirring while cooling. |
| 60-----                 | 180                                   | 5.0                            | 0.16                                                                                    | 45                       | 43    | 2:1                             | 21                  | 6.6                                        | 6.4     | —           | 5½                                  | 5          | 0        | 10     | Do.                                                                        |
| 40-----                 | 200                                   | 5.0                            | 0.16                                                                                    | 45                       | 43    | 2:1                             | 65                  | 5.5                                        | —       | —           | 4½                                  | 4½         | 0        | 3      | Mix aged 42 days.                                                          |
| 60-----                 | 180                                   | 5.0                            | 0.16                                                                                    | 45                       | 43    | 2:1                             | 51                  | 6.7                                        | —       | —           | 5½                                  | 5          | 0        | 1      | Do.                                                                        |

## EXAMPLE 9

This example illustrates the use of other 70 metallic oxides, more particularly bismuth tri-oxide and stannic oxide, instead of antimony trioxide in the treating compositions. The vinyl chloride copolymer (used in the form of an aqueous dispersion) was the same Geon copolymer

was done in pint jars, each of which contained a 6-inch square sample of fabric, 20 steel balls and 200 ml. of a 0.5% neutral soap solution heated to 180° F. The jars were revolved for 5 minutes. See Table VIII for additional details of the treatment and the results obtained.

Table VIII

| Conditions of Curing |    | Weight Ratio of Copolymer to Titanium Dioxide | Per Cent Vinyl Chloride Copolymer in Bath | Per Cent Titanium Dioxide in Bath | Per Cent Total Add-On |        | Flame Test Vertical Charred Length, Inches |          |          |
|----------------------|----|-----------------------------------------------|-------------------------------------------|-----------------------------------|-----------------------|--------|--------------------------------------------|----------|----------|
|                      |    |                                               |                                           |                                   | Bath 1                | Bath 2 | 1 Wash                                     | 3 Washes | 5 Washes |
| 140                  | 40 | 1:1                                           | 2.5                                       | 2.5                               | 20                    | 3      | 5                                          | 4 1/4    | 5        |
| 140                  | 40 | 1:1                                           | 5.0                                       | 5.0                               | 19                    | 8      | 5 1/2                                      | 5 1/4    | 5 1/4    |
| 160                  | 15 | 1:1                                           | 5.0                                       | 5.0                               | 17                    | 11     | 6                                          | 5        | 5 1/4    |
| 140                  | 40 | 1:1                                           | 7.5                                       | 7.5                               | 18                    | 14     | 6                                          | 5 1/2    | 5 1/2    |
| 160                  | 15 | 1:1                                           | 7.5                                       | 7.5                               | 19                    | 18     | 5 1/4                                      | 6 1/4    | 6        |
| 140                  | 40 | 1:1                                           | 2.5                                       | 2.5                               | 24                    | 0      | 4 1/4                                      | 6        | 6 1/4    |
| 140                  | 40 | 1:1                                           | 5.0                                       | 5.0                               | 28                    | 0      | 4 1/4                                      | 5 1/4    | 5 1/4    |
| 160                  | 15 | 2:1                                           | 5.0                                       | 2.5                               | 33                    | 0      | 5 1/2                                      | 6        | 6        |

## EXAMPLE 11

In this example ammonium dicyanamide or ammonium cyanate was used as the water-soluble nitrogenous substance and monosodium or disodium phosphate as the water-soluble oxygen-containing acid of phosphorus. The metallic

strength of the untreated and treated cotton sheeting and rayon suiting, and the results of flame tests on both kinds of treated goods after being rinsed and after the aforementioned washes. The rinsed and washed samples were pressed dry before testing.

Table X

|                                      | Weight Retention Tests (Wt. Retained, Per Cent) |        |            |            |            | Horizontal Flame Tests (Avg. Diam. of Burned Area in In.) |            |            |            | Vertical Flame Tests (Ht. of Burned Area in In.) |            |            |            | Total Tensile Strength (In Pounds) |
|--------------------------------------|-------------------------------------------------|--------|------------|------------|------------|-----------------------------------------------------------|------------|------------|------------|--------------------------------------------------|------------|------------|------------|------------------------------------|
|                                      | Per Cent Applied                                | Rinsed | 1 Hr. Wash | 3 Hr. Wash | 5 Hr. Wash | Rinsed                                                    | 1 Hr. Wash | 3 Hr. Wash | 5 Hr. Wash | Rinsed                                           | 1 Hr. Wash | 3 Hr. Wash | 5 Hr. Wash |                                    |
| 100 x 60 Cotton Sheetings, Untreated |                                                 |        |            |            |            | C                                                         |            |            |            | C                                                |            |            |            |                                    |
| 100 x 60 Cotton Sheetings, Treated:  |                                                 |        |            |            |            |                                                           |            |            |            |                                                  |            |            |            | 137                                |
| 5' cure                              | 38                                              | 28     | 18         | 14         | 13         | 2.4                                                       | 2.5        | 2.4        | 2.5        | 3.3                                              | 3.3        | 2.9        | 2.8        | 132                                |
| 10' cure                             | 39                                              | 27     | 21         | 18         | 16         | 2.4                                                       | 2.4        | 2.4        | 2.4        | 3.2                                              | 3.3        | 2.8        | 2.7        | 126                                |
| 15' cure                             | 40                                              | 28     | 21         | 16         | 14         | 2.4                                                       | 2.4        | 2.4        | 2.4        | 3.3                                              | 3.1        | 2.8        | 2.9        | 130                                |
| Rayon Suiting, Untreated             |                                                 |        |            |            |            | C                                                         |            |            |            | C                                                |            |            |            |                                    |
| Rayon Suiting, Treated:              |                                                 |        |            |            |            |                                                           |            |            |            |                                                  |            |            |            |                                    |
| 5' cure                              |                                                 |        |            |            |            | 1.8                                                       | 1.9        | 1.8        | 1.8        | 2.5                                              | 2.8        |            |            | 237                                |
| 10' cure                             |                                                 |        |            |            |            | 1.8                                                       | 1.9        | 1.8        | 1.8        | 2.6                                              | 2.6        |            |            | 239                                |
| 15' cure                             |                                                 |        |            |            |            | 1.8                                                       | 1.9        | 1.8        | 1.8        | 2.5                                              | 2.5        | 2.7        | 2.5        | 233                                |
|                                      |                                                 |        |            |            |            |                                                           |            |            |            |                                                  |            |            |            | 231                                |

C—Complete charring of sample.

oxide was antimony trioxide and the halogen-containing thermoplastic substance was a vinyl chloride copolymer such as was employed in prior examples. The ingredients were applied by a two-bath process, the second bath being an aqueous dispersion containing, by weight, 5.8% of  $Sb_2O_3$  and 11% of the aforementioned copolymer. Further information on the treatment and the results obtained appears in Table IX.

It will be noted from Table X that the results of flame-resistance tests were excellent at all of the cure times employed and that the loss in tensile strength, if any, of each of the treated fabrics was very little; and that in one case (treated rayon suiting using a 5-minute cure) there was an actual gain in tensile strength.

The treated fabrics were analyzed for phosphorus. The results are shown in Table XI.

Table IX

| Nitrogenous Substance | Salt                 | Weight Ratio of Nitrogenous Substance to Salt | Per Cent Dry Total Add-On |        | pH First Bath | pH Rinsings | Flame Tests                     |                       |        |          | Phosphorus as Per Cent $H_3PO_4$ |
|-----------------------|----------------------|-----------------------------------------------|---------------------------|--------|---------------|-------------|---------------------------------|-----------------------|--------|----------|----------------------------------|
|                       |                      |                                               | Bath 1                    | Bath 2 |               |             | Vertical Charred Length, Inches | Time After Glow, Sec. | 1 Wash | 5 Washes |                                  |
| Ammonium dicyanamide  | Disodium phosphate   | 1:1.45                                        | 10                        | 19     | 6.8           | 4.9         | 4                               | 4                     | 0      | 1        |                                  |
| Do.                   | Monosodium phosphate | 1:1.2                                         | 19                        | 19     | 6.1           | 4.7         | 6                               | 0                     | 0      | 2        |                                  |
| Ammonium cyanate      | Disodium phosphate   | 1:1.45                                        | 15                        | 19     | 9.1           | 8.5         | 4 1/2                           | 4 1/2                 | 4      | 10       |                                  |
| Do.                   | Monosodium phosphate | 1:1.2                                         | 15                        | 18     | 6.2           | 6.4         | 3 1/2                           | 4 1/2                 | 5      | 10       |                                  |

## EXAMPLE 12

The treating composition used in this example was essentially the same as that described under Example 1. The aqueous dispersion contained approximately 57% by weight of solids. Heavy rayon suiting and 100 x 60 cotton sheeting were padded through the dispersion, dried at about 104.5° C. and then cured by heating for 5, 10 or 15 minutes at 160° C. Table X gives the weight-retention values of the cured samples of cotton sheeting as initially produced, after being rinsed in warm water and after washing for 1, 3 and 5 hours in a 0.1% soap solution at 160° F. in the case of the cotton sheeting and at 100° F. in the case of the rayon suiting, as well as the tensile

strength of the untreated and treated cotton sheeting and rayon suiting, and the results of flame tests on both kinds of treated goods after being rinsed and after the aforementioned washes. The rinsed and washed samples were pressed dry before testing.

Table XI

| Fabric Treated and Cure Times | Phosphorus as Per Cent $H_3PO_4$ |             |
|-------------------------------|----------------------------------|-------------|
|                               | Rinsed Original                  | 6 Hour Wash |
| 100 x 60 Cotton Sheetings:    |                                  |             |
| 5' cure                       | 6.6                              | 6.5         |
| 10' cure                      | 6.7                              | 6.7         |
| 15' cure                      | 6.7                              | 6.7         |
| Rayon Suiting:                |                                  |             |
| 5' cure                       | 7.9                              | 7.6         |
| 10' cure                      | 7.8                              | 7.7         |
| 15' cure                      | 7.8                              | 7.6         |

From Table XI it will be seen that the phosphorus content of the treated fabric remains substantially constant on prolonged washing of the fabric in a soap solution.

EXAMPLE 13

This example illustrates the results obtained with various concentrations (57%, 42.6% and 28.5% solids) of the same treating ingredients in the same proportions used in the treating composition of the prior example in imparting flame resistance to different fabrics, more particularly to 100 x 60 untreated cotton cloth, cotton marquisette, rayon challis and rayon netting. The wet pick-up was approximately 80% by weight of the dry fabric, in the case of the cotton goods, about 100% by weight of the dry fabric, in the case of the rayon challis and about 150%, by weight of the dry fabric, in the case of the rayon netting. The time of curing was 5 minutes at 160° F. The time of curing was 5 minutes at 160° C.

It will be noted in Table XII that the treatment of the rayon netting resulted, in all cases, in a substantial increase in the tensile strength of the treated fabric as compared with the untreated netting, the percentage increase being more than 21%. This was quite surprising and unexpected, and in no way could have been predicted.

EXAMPLE 14

The treating composition used in this example was essentially the same as that employed in Examples 1 and 12. The aqueous dispersion was applied to various cotton fabrics by a one-bath process. Drying and curing of the treated fabrics were carried out under essentially the same conditions described in the prior example. The treated fabrics were given 5 washes of 1 hour each in a 0.1% soap solution at 160° F. The results are shown in Table XIII.

Table XIII

| Material Treated               | Flame Tests             |      |                     |      |                         |      |                     |      | Tensile Strength in Pounds |      |  |  |
|--------------------------------|-------------------------|------|---------------------|------|-------------------------|------|---------------------|------|----------------------------|------|--|--|
|                                | Before Washing          |      |                     |      | After Washing           |      |                     |      |                            |      |  |  |
|                                | Avg. After-Glow in Sec. |      | Avg. Char in Inches |      | Avg. After-Glow in Sec. |      | Avg. Char in Inches |      |                            |      |  |  |
|                                | Warp                    | Fill | Warp                | Fill | Warp                    | Fill | Warp                | Fill | Warp                       | Fill |  |  |
| Untreated Duck                 |                         |      |                     |      |                         |      |                     |      | 187                        | 137  |  |  |
| Treated Duck                   | 2                       | 3    | 2.75                | 2.8  | 13                      | 13   | 3.35                | 3.5  | 166                        | 129  |  |  |
| Untreated Marquisette          |                         |      |                     |      |                         |      |                     |      | 21                         | 11   |  |  |
| Treated Marquisette            | 0                       | 0    | 5.1                 | 4.7  | 0                       | 0    | 5.1                 | 5.85 | 18                         | 6    |  |  |
| Untreated white flock          |                         |      |                     |      |                         |      |                     |      | 47                         | 35   |  |  |
| Treated white flock            | 0                       | 1    | 3.7                 | 3.75 | 0                       | 2    | 3.8                 | 4.35 | 40                         | 27   |  |  |
| Untreated unbleached muslin    |                         |      |                     |      |                         |      |                     |      | 47                         | 33   |  |  |
| Treated unbleached muslin      | 0                       | 0    | 3.5                 | 3.5  | 1                       | 1    | 4.75                | 4.8  | 44                         | 30   |  |  |
| Untreated flowered herringbone |                         |      |                     |      |                         |      |                     |      | 108                        | 63   |  |  |
| Treated flowered herringbone   | 1-2                     | 2    | 3.25                | 3.0  | 4                       | 4    | 4.6                 | 4.15 | 93                         | 55   |  |  |
| Untreated maroon herringbone   |                         |      |                     |      |                         |      |                     |      | 118                        | 47   |  |  |
| Treated maroon herringbone     | 1-2                     | 1    | 3.7                 | 3.7  | 3                       | 7.0  | 4.0                 | 4.3  | 111                        | 42   |  |  |
| Untreated white twill jean     |                         |      |                     |      |                         |      |                     |      | 101                        | 53   |  |  |
| Treated white twill jean       | 1                       | 0    | 3.8                 | 3.5  | 2                       | 1    | 4.15                | 3.6  | 70                         | 52   |  |  |

The other conditions of treating and testing were the same as in Example 12. The results of flame tests and tensile strength tests are given in Table XII.

EXAMPLE 15

This example illustrates the results obtained using polymeric vinyl chloride (polyvinyl chlo-

Table XII

|                                                           | Horizontal Flame Tests (Av. dia. of burned area/in.) |            |            |            | Vertical Flame Tests (Ht. of burned area in inches) |            |            |            | Total Tensile Strength (In Pounds) |
|-----------------------------------------------------------|------------------------------------------------------|------------|------------|------------|-----------------------------------------------------|------------|------------|------------|------------------------------------|
|                                                           | Rinsed                                               | 1 Hr. Wash | 3 Hr. Wash | 5 Hr. Wash | Rinsed                                              | 1 Hr. Wash | 3 Hr. Wash | 5 Hr. Wash |                                    |
|                                                           | C                                                    | -----      | -----      | -----      | C                                                   | -----      | -----      | -----      |                                    |
| 100 x 60 Cotton Cloth, Untreated                          | C                                                    | -----      | -----      | -----      | C                                                   | -----      | -----      | -----      | 159                                |
| 100 x 60 Cotton Cloth, treated 57% solids in pad liquor   | 2.2                                                  | 2.3        | 2.8        | 2.8        | 3.4                                                 | 3.2        | 3.1        | 3.4        | 147                                |
| 100 x 60 Cotton Cloth, treated 28.5% solids in pad liquor | 3.7                                                  | 3.2        | 2.8        | 2.7        | 4.3                                                 | 4.0        | 4.3        | 4.2        | 140                                |
| 100 x 60 Cotton Cloth, treated 42.6% solids in pad liquor | 2.4                                                  | 2.4        | 2.4        | 2.4        | 3.4                                                 | 3.2        | 3.3        | 3.7        | 142                                |
| Cotton marquisette, Untreated                             | C                                                    | -----      | -----      | -----      | C                                                   | -----      | -----      | -----      | 54                                 |
| Cotton marquisette, treated 57% solids in pad liquor      | 2.1                                                  | 2.2        | 2.2        | 2.3        | 3.5                                                 | 3.8        | 3.5        | 3.0        | 40                                 |
| Cotton marquisette, treated 42.6% solids in pad liquor    | 2.2                                                  | 2.2        | 2.3        | 2.4        | 3.8                                                 | 3.6        | 3.6        | 4.3        | 43                                 |
| Rayon Challis, Untreated                                  | C                                                    | -----      | -----      | -----      | C                                                   | -----      | -----      | -----      | 138                                |
| Rayon Challis, treated 57% solids in pad liquor           | 2.1                                                  | 2.1        | 2.1        | 2.1        | 3.3                                                 | 3.5        | 3.4        | 3.2        | 130                                |
| Rayon Challis, treated 42.6% solids in pad liquor         | 2.2                                                  | 2.3        | 2.3        | 2.2        | 3.6                                                 | 3.8        | 3.3        | 3.5        | 141                                |
| Rayon Challis, treated 28.5% solids in pad liquor         | 2.6                                                  | 2.7        | 2.8        | 2.7        | 4.1                                                 | 3.1        | 3.9        | 4.3        | 137                                |
| Rayon netting, Untreated                                  | C                                                    | -----      | -----      | -----      | C                                                   | -----      | -----      | -----      | 42                                 |
| Rayon netting, treated 57% solids in pad liquor           | 1.9                                                  | -----      | 2.0        | 2.0        | 3.3                                                 | 3.4        | 3.4        | 3.3        | 52                                 |
| Rayon netting, treated 42.6% solids in pad liquor         | 1.9                                                  | -----      | 2.0        | 2.0        | 3.2                                                 | 3.3        | 3.2        | 3.7        | 51                                 |
| Rayon netting, treated 28.5% solids in pad liquor         | 2.1                                                  | -----      | 2.0        | 2.0        | 3.8                                                 | 3.3        | 3.3        | 3.8        | 61                                 |

C—Complete charring of sample.

ride) as the halogen-containing thermoplastic substance and applying the treating composition to 80 x 80 cotton cloth by one-bath and two-bath processes in essentially the same manner as previously has been described.

*One-bath process*  
COMPOSITION OF BATH

|                                                                                                                                    | Parts<br>(approx.) |  |
|------------------------------------------------------------------------------------------------------------------------------------|--------------------|--|
| Monoguanidine phosphate                                                                                                            |                    |  |
| Urea                                                                                                                               | 151.0              |  |
| Hexamethylene tetramine                                                                                                            | 282.0              |  |
| Antimony trioxide introduced in the form of an aqueous dispersion prepared as described under Example 1                            | 20.0               |  |
| Polyvinyl chloride introduced in the form of an aqueous dispersion                                                                 | 56.0               |  |
| Dispersing agent used in dispersing the antimony trioxide                                                                          | 50.0               |  |
| Water, including that used in dispersing the antimony trioxide and the polyvinyl chloride                                          | 1.5                |  |
| Essentially the same procedure was followed in applying the composition to 80 x 80 cotton cloth as that described under Example 1. | 20                 |  |

*Two-bath process*  
COMPOSITION OF BATH 1

|                         | Parts<br>(approx.) |  |
|-------------------------|--------------------|--|
| Monoguanidine phosphate |                    |  |
| Urea                    | 151                |  |
| Hexamethylene tetramine | 282                |  |
| Water                   | 20                 |  |

COMPOSITION OF BATH 2

|                                                                                                         | Parts<br>(approx.) |  |
|---------------------------------------------------------------------------------------------------------|--------------------|--|
| Antimony trioxide introduced in the form of an aqueous dispersion prepared as described under Example 1 |                    |  |
| Polyvinyl chloride introduced in the form of an aqueous dispersion                                      | 56.0               |  |
| Dispersing agent used in dispersing the antimony trioxide                                               | 50.0               |  |
| Water, including that used in dispersing the antimony trioxide and the polyvinyl chloride               | 1.5                |  |

Essentially the same procedure was followed in applying the compositions of Baths 1 and 2 to 80 x 80 cotton as described under Example 2. Further information on the treatment and on the results obtained appears in Table XIV.

Table XIV

| Per Cent Total Dry Add-On | Flame Tests, Vertical Charred Length, Inches |                               |                               |          | Average Per Cent Loss In Tensile Strength |
|---------------------------|----------------------------------------------|-------------------------------|-------------------------------|----------|-------------------------------------------|
|                           | Bath 1                                       | Bath 2                        | 1 Wash                        | 5 Washes |                                           |
| 27                        | ( <sup>1</sup> ) 16                          | 3 <sup>1</sup> / <sub>2</sub> | 4 <sup>1</sup> / <sub>2</sub> |          | -9                                        |
| 15                        |                                              | 3 <sup>1</sup> / <sub>2</sub> | 4 <sup>1</sup> / <sub>2</sub> |          | -12                                       |

<sup>1</sup> All in one bath.

EXAMPLE 16

This example illustrates the results obtained when hexamethylene tetramine and other basic materials were used as components of the treating composition.

Compositions were prepared in essentially the

same manner as described under Example 1, using the following proportions of ingredients:

|                         | Parts |
|-------------------------|-------|
| Monoguanidine phosphate | 75.5  |
| Urea                    | 141.0 |
| Basic material          | 10.0  |
| Water                   | 160.0 |

Aqueous dispersion containing about 55.5% by weight of a vinyl chloride copolymer such as described under Example 1. 45.5

Aqueous dispersion containing about 41% by weight of  $Sb_2O_3$  and about 1.3% by weight of a dispersing agent, more particularly a sodium salt of a condensation product of formaldehyde and a naphthalene sulfonic acid (Tanol P). 68.0

The following basic substances were employed in individual compositions:

1. Triethylene tetramine.
2. Tetraethylene pentamine.
3. Hexamethylene tetramine.
4. Calcium carbonate in the form of a 40% aqueous dispersion using 0.5% of the aforementioned dispersing agent and water from the 160 parts mentioned in the formula.

Essentially the same procedure was employed in applying the composition to 80 x 80 cotton cloth as that described under Example 1. Further information on the treatment and on the results obtained appears in Table XV.

Table XV

| Basic substance                                   | 1   | 2   | 3   | 4   |
|---------------------------------------------------|-----|-----|-----|-----|
| Per cent wet pick-up                              | 120 | 126 | 127 | 121 |
| Per cent total dry add-on                         | 29  | 30  | 33  | 31  |
| pH of bath                                        | 6.3 | 6.3 | 5.7 | 5.5 |
| pH of rinsings                                    | 6.7 | 6.5 | 6.1 | 6.6 |
| Average per cent loss or gain in tensile strength | -2  | 0   | +3  | -3  |
| Vertical flame tests:                             |     |     |     |     |
| Charred length in inches:                         |     |     |     |     |
| 1 wash                                            | 4.3 | 4.2 | 4.0 | 4.3 |
| 5 washes                                          | 4.8 | 4.1 | 4.4 | 4.4 |
| After glow in seconds:                            |     |     |     |     |
| 1 wash                                            | 7   | 8   | 7   | 6   |
| 5 washes                                          | 19  | 15  | 20  | 16  |

It will be understood, of course, by those skilled in the art that our invention is not limited to the particular ingredients, proportions thereof and application methods described in the above illustrative examples. As has been mentioned hereinbefore, the water-soluble nitrogenous substance may be urea, biuret, ammonium cyanate, ammonium dicyanimide, or mixtures thereof, that is, mixtures of any or all of these substances in any proportions. We prefer to use urea as the water-soluble nitrogenous substance.

Any water-soluble salt of an oxygen-containing acid of phosphorus wherein the phosphorus atom has a valence of 5, numerous examples of which have been given earlier herein, may be used. Mixtures of such salts may be employed as well as salts of mixtures of such acids which include orthophosphoric acid, metaphosphoric acid and pyrophosphoric acid, the mixed acids being sometimes collectively designated as "polyphosphoric" acid.

Any of the oxides of tin, titanium, antimony or busmuth, or any mixtures of any of the oxides of these metals, in any proportions, may be employed. These oxides may act catalytically to accelerate dehalogenation of the thermally unstable, halogen-containing thermoplastic substance and to promote more rapid hydrohalide (i. e., hydrogen halide) formation at tempera-

tures near that at which thermal decomposition of the cellulosic material occurs. We prefer to use an oxide of antimony, more particularly antimony trioxide, as the metallic oxide.

The thermoplastic substance may be any thermoplastic material (e. g., a vinyl resin, more particularly a vinyl halide polymerization product) containing at least 20%, more particularly at least 30% and preferably at least 40%, by weight of combined halogen (e. g., chlorine, bromine, etc.) and which is capable of rupturing under heat at carbon-halogen bonds, numerous examples of which materials have been given hereinbefore. Additional examples include the halogenated diphenyls (e. g., pentachlorodiphenyl, pentabromodiphenyl, etc.) and the halogenated (e. g., chlorinated, brominated, etc.) naphthalenes, which compounds contain at least 20% by weight of combined chlorine, bromine or other halogen. We prefer to use polyvinyl chloride or a vinyl chloride copolymer containing at least 80% by weight of combined (i. e., combined in the copolymer molecule) vinyl chloride, more particularly a copolymer of, by weight, from about 80% to about 99% of vinyl chloride and from about 20% to about 1% of an acrylic ester, specifically an alkyl acrylate such, for instance, as methyl, ethyl, propyl or butyl acrylate.

It is important that the water-soluble nitrogenous substance, the water-soluble salt of an oxygen-containing acid of phosphorus, the metallic oxide and the halogen-containing thermoplastic substance be used in proportions within the ranges given in the eighth paragraph of this specification. As shown by the numerous examples, especially in the tables, the proportions may be considerably varied within these broader ranges and still obtain a finished textile which is resistant to flame even after numerous laundering or dry-cleaning operations and without excessive tendering (in many cases without any tendering) of the textile. Furthermore, by using the ingredients within the proportions stated hereinbefore, a flame-resistant textile having a good hand or feeling to the touch is obtained. As will be readily appreciated by those skilled in the textile art, the matter of hand or feeling to the touch is, for most applications, of considerable importance from both saleability and utility standpoints.

The fundamental treating compositions of this invention may be modified by incorporating therein various modifying agents which aid in further improving the flame-resistant characteristics of the treated cellulosic material or which facilitate the technique of application. For instance, the compositions may also contain minor amounts (e. g., from 1 to 30% by weight of the total solids content) of such glow retardants as the glow-retarding borates, phosphates, pyrophosphates, etc., e. g., zinc borate, zinc phosphate, zinc ammonium phosphate, stannic phosphate, phenyl diamido phosphate, melamine pyrophosphate, etc. Agents which have a buffering effect on the composition after being applied to the fabric or other textile, e. g., calcium carbonate, magnesium oxide, hexamethylene tetramine and other polyalkylene polyamines, etc., may be incorporated into the treating compositions as desired or as conditions may require.

The pH of the bath containing the ingredients of (B) in a two-bath process or the bath containing all of the ingredients in a one-bath process should be adjusted to a pH (glass electrode pH) within the range of from about 3 to about

10, e. g., a pH of from about 3½ or 4 to about 7 or 8, if the pH of the aqueous composition containing these ingredients (water-soluble salt of the oxygen-containing acid of phosphorus and water-soluble nitrogenous substance) is not initially within a pH range of from about 3 to about 10. Preferably the pH of the aqueous composition containing the ingredients of (B) is between 4 and 7, e. g., about 6.

The present invention is applicable to the production of a wide variety of flame-resistant cellulosic materials, e. g., wearing apparel of all kinds, especially children's clothes and clothing used by the armed forces, curtains, draperies, sheeting, furniture coverings, linings for electric blankets, net fabrics, non-woven fabrics, chenilles, etc., and which are made of cellulosic materials such as are described in the first paragraph of this specification and elsewhere herein. Other applications of the flame-resistant products of our invention include those described in Chapters VII and VIII of the aforementioned book, edited by Little, entitled "Flameproofing Textile Fabrics."

The terms "flame resistance" and "flame-resistant" as used herein and in the appended claims with reference to cellulosic materials, specifically cellulosic textiles, are used generically to include within their meanings treated cellulosic materials (e. g., treated fabrics) which, after ignition, will continue to burn at a relatively slow rate as well as those which, after ignition, will burn over only a limited area beyond that directly exposed to the source of ignition and which may be specifically designated as "fire-resistant" cellulosic materials. It will be apparent from the examples herein given that most of the products of our invention properly fall within the specific classification of fire-resistant cellulosic materials.

The terms "textile" and "textile material" as used generically herein and in the appended claims include within their meaning filaments, fibers, rovings, slivers, threads, yarns, twisted yarns, etc., as such or in woven, felted or otherwise formed fabrics, sheets, cloths and the like.

We claim:

1. A method of imparting flame-resistance to a cellulosic textile material of the class consisting of natural celluloses, regenerated celluloses and mixtures thereof, said method comprising impregnating said material with an association of (1) an aqueous liquid composition having a pH of from about 3 to about 10 and containing (a) ingredients initially in the form of a water-soluble salt of an oxygen-containing acid of phosphorus wherein the phosphorus atom has a valence of 5 and a water-soluble nitrogenous substance selected from the group consisting of urea, blucret, ammonium cyanate, ammonium dicyanamide and mixtures thereof, said salt of an oxygen-containing acid of phosphorus and said nitrogenous substance being employed in a weight ratio of 1 part of the former calculated as  $H_3PO_4$  to from 1 to 20 parts of the latter, and (2) an aqueous liquid composition containing (b) ingredients comprising a finely divided, oxygen-containing substance of the group consisting of tin, titanium, antimony and bismuth oxides and mixtures thereof, and a thermoplastic halogen-containing, organic substance having at least 20% by weight of combined halogen and capable of rupturing under heat at carbon-halogen bonds, said finely divided oxygen-containing substance and

said thermoplastic substance being employed in a weight ratio of 1 part of the former to from 0.6 to 20 parts of the latter, and the said ingredients of (a) and (b) being employed in a weight ratio of 1 part of the latter to from 0.2 to 8 parts of the former; heating the textile material after it has been impregnated with a composition comprising the aqueous liquid composition of (1) at a temperature within the range of about 135° C. to about 200° C.; and washing the resulting material to remove any residual water-soluble substances therefrom, the total amount of the compositions of (1) and (2) with which the cellulosic material initially is impregnated being such that the finished flame-resistant textile contains from about 10% to about 75% by weight, based on the dry weight of the untreated textile, of washfast impregnant.

2. The process of claim 1 wherein the aqueous composition of (1) and the aqueous composition of (2) are applied simultaneously in a single bath.

3. A method as in claim 1 wherein the cellulosic textile material is a cotton textile material.

4. A method as in claim 1 wherein the cellulosic textile material is a viscose rayon textile material.

5. A flame-resistant cellulosic material of the class consisting of natural celluloses, regenerated celluloses and mixtures thereof, resulting from the method of claim 1.

6. An aqueous dispersion, suitable for use in imparting flame-resistance to cellulosic textile materials selected from the group consisting of natural celluloses, regenerated celluloses and mixtures thereof, having a pH of from about 3 to about 10 and comprising (1) a finely divided, oxygen-containing substance of the group consisting of tin, titanium, antimony and bismuth oxides and mixtures thereof and (2) a thermoplastic halogen-containing organic substance containing at least 20% by weight of combined halogen and capable of rupturing under heat at carbon-halogen bonds, the ingredients of (1) and (2), which together are designated hereinafter as (A), being employed in a weight ratio of 1 part of the former to from 0.6 to 20 parts of the latter and being dispersed in water containing ingredients initially in the form of (3) a water-soluble salt of an oxygen-containing acid of phosphorus wherein the phosphorus atom has a valence of 5 and (4) a water-soluble nitrogenous substance of the group consisting of urea, biuret, ammonium cyanate, ammonium dicyanamide, and mixtures thereof, the ingredients of (3) and (4), which together are designated hereinafter as (B), being employed in a weight ratio of 1 part of the former calculated as  $H_3PO_4$  to from 1 to 20 parts of the latter, and the ingredients of (A) and (B) being employed in a weight ratio of 1 part of the former to from 0.2 to 8 parts of the latter.

7. The aqueous dispersion of claim 6 wherein the finely divided oxygen-containing substance is antimony trioxide, the thermoplastic halogen-containing organic substance is a vinyl chloride polymerization product, the water-soluble salt of an oxygen-containing acid of phosphorus is monoguanidine phosphate and the water-soluble nitrogenous substance is urea.

8. A method of imparting flame-resistance to a textile material comprising fibers of a cellulosic material of a class consisting of natural celluloses, regenerated celluloses and mixtures thereof, said method comprising impregnating said

textile material with the composition of claim 6, drying the impregnated material, heating the dried material at a temperature within the range of 135° C. to 200° C. and washing the resulting material to remove any residual water-soluble substances therefrom, the total amount of said ingredients of (A) and (B) with which the cellulosic textile material initially is impregnated being such that the finished flame-resistant textile contains from about 10% to about 50% by weight, based on the dry weight of the untreated textile, of washfast impregnant.

9. A method of imparting flame-resistance to a textile comprising fibers of a cellulosic material of the class consisting of natural celluloses, regenerated celluloses and mixtures thereof, said method comprising impregnating said textile with an aqueous dispersion having a pH within the range of 3 to 10 and comprising (1) a finely divided oxide of antimony and (2) a thermoplastic vinyl chloride polymerization product containing at least 40% by weight of combined chlorine, the ingredients of (1) and (2), which together are designated hereinafter as (A), being employed in a weight ratio of 1 part of the former to from 0.6 to 20 parts of the latter and being dispersed in water containing ingredients initially in the form of (3) a water-soluble guanidine phosphate and (4) urea, the ingredients of (3) and (4), which together are designated hereinafter as (B), being employed in a weight ratio of 1 part of the former calculated as  $H_3PO_4$  to from 2 to 20 parts of the latter, and the ingredients of (A) and (B) being employed in a weight ratio of 1 part of the former to from 0.2 to 8 parts of the latter, drying the impregnated material, heating the dried material at a temperature within the range of 135° C. to 200° C., and washing the resulting material to remove any residual water-soluble substances therefrom, the total amount of the ingredients of (A) and (B) with which the cellulosic textile material initially is impregnated being such that the finished flame-resistant textile contains from about 10% to about 75% by weight, based on the dry weight of the untreated textile, of washfast impregnant.

10. A flame-resistant textile material of the class consisting of natural celluloses, regenerated celluloses and mixtures thereof, resulting from the method of claim 9.

11. A method as in claim 9 wherein the water-soluble guanidine phosphate of (3) is monoguanidine phosphate.

12. A method as in claim 9 wherein the aqueous dispersion also contains a small amount, not exceeding about 7% by weight of the ingredients of (B), of a polyalkylene polyamine having a boiling point substantially above 200° C.

13. A method of imparting flame-resistance to a textile comprising fibers of a cellulosic material of the class consisting of natural celluloses, regenerated celluloses and mixtures thereof, said method comprising impregnating said textile with an aqueous solution having a pH within the range of from 3 to 10 and containing ingredients initially in the form of (1) a water-soluble salt of an oxygen-containing acid of phosphorus wherein the phosphorus atom has a valence of 5 and (2) a water-soluble nitrogenous substance of the group consisting of urea, biuret, ammonium cyanate, ammonium dicyanamide and mixtures thereof, the ingredients of (1) and (2), which together are designated hereinafter as (B), being employed in a weight ratio

70

of 1 part of the former calculated as  $H_3PO_4$  to from 1 to 20 parts of the latter; heating the impregnated textile at a temperature within the range of 135° C. to 200° C.; washing the resulting textile to remove any residual water-soluble substances therefrom; impregnating the heated and washed textile with ingredients comprising (3) a finely divided, oxygen-containing substance of the group consisting of tin, titanium, antimony and bismuth oxides and mixtures thereof and (4) a thermoplastic halogen-containing organic substance containing at least 20% by weight of combined halogen and capable of rupturing under heat at carbon-halogen bonds, the ingredients of (3) and (4), which together are designated hereinafter as (A), being employed in a weight ratio of 1 part of the former to from 0.6 to 20 parts of the latter, the ingredients of (A) and (B) being employed in a weight ratio of 1 part of the former to from 0.2 to 8 parts of the latter, and the total amount of the ingredients of (A) and (B) with which the said textile is impregnated being such that the finished flame-resistant textile contains from about 10% to about 75% by weight, based on the dry weight of the untreated textile, of washfast impregnant.

14. A flame-resistant cellulosic material of the class consisting of natural celluloses, regenerated celluloses and mixtures thereof, resulting from the method of claim 13.

15. The method of claim 13 wherein the water-soluble salt of an oxygen-containing acid of phosphorus is a guanidine phosphate, the water-soluble nitrogenous substance is urea, the finely divided oxygen-containing substance is antimony trioxide and the thermoplastic halogen-containing substance is a vinyl resin containing at least 40% by weight of combined chlorine.

16. A method as in claim 15 wherein the textile is a cotton fabric material.

17. A method as in claim 15 wherein the water-soluble guanidine phosphate is monoguanidine phosphate.

ANNE MACMILLAN LOUKOMSKY.  
ROY H. KIENLE.  
THEODORE F. COOKE.

## REFERENCES CITED

The following references are of record in the file of this patent:

## UNITED STATES PATENTS

|    | Number    | Name           | Date           |
|----|-----------|----------------|----------------|
| 25 | 2,089,697 | Groebe         | Aug. 10, 1937  |
|    | 2,178,825 | Clayton et al. | Nov. 7, 1939   |
|    | 2,357,725 | Bennett        | Sept. 5, 1944  |
|    | 2,413,163 | Bacon          | Dec. 24, 1946  |
|    | 2,427,997 | White          | Sept. 23, 1947 |
| 30 | 2,461,538 | Fischer        | Feb. 15, 1949  |